

Oct. 13, 1931.

P. A. E. ARMSTRONG

1,826,860

PROCESS OF MAKING PRODUCTS WITH WELDED FACES OF STABLE SURFACE ALLOY

Filed Jan. 16, 1924

Fig 1



Fig 2



Fig 3



Fig 4



INVENTOR

P.A.E. Armstrong

BY *H. H. Dyke*

ATTORNEY

## UNITED STATES PATENT OFFICE

PERCY A. E. ARMSTRONG, OF LOUDONVILLE, NEW YORK, ASSIGNOR TO LUDLUM STEEL COMPANY, OF WATERVLIET, NEW YORK, A CORPORATION OF NEW JERSEY

## PROCESS OF MAKING PRODUCTS WITH WELDED FACES OF STABLE SURFACE ALLOY

Continuation of application Serial No. 527,225, filed January 5, 1922, this application filed January 16, 1924, Serial No. 686,654.

My invention relates to a process of making products with welded faces of stable surface alloy.

The present application is a continuation 5 of my prior copending application Serial No. 527,225, filed Jan. 5, 1922.

According to the present invention I weld stable surface alloy as disclosed, for example, in my U. S. Patent No. 1,322,511 of Nov. 25, 10 1919, or other stable surface alloy material, such, for example, as so-called stainless steel or stainless iron, to relatively base metal, such as ordinary low carbon steel or iron, by casting the stable surface alloy against a thin 15 section of the base metal, which becoming highly heated when the stable surface alloy is cast against it becomes welded thereto, and thereafter cast additional base metal against the base metal previously welded to the stable 20 surface alloy, and the base metal parts being thus welded together produce an ingot or the like having substantial thicknesses of base metal with a face of stable surface alloy, which can be drawn, rolled or formed into 25 products, articles and shapes as desired. The stable surface alloy face so obtained is securely and permanently welded and united to the base backing in the manner described.

I have shown modes of carrying out my invention in the accompanying drawings, but it is to be understood that same are only for illustration and for affording an understanding of the invention.

In said drawings, Fig. 1 is a cross-sectional view indicating the casting in a ingot mold of stable surface alloy about two thin sections of base metal arranged back to back. Fig. 2 is a similar view indicating the casting of Fig. 1 separated into parts with the 35 base metal sides inwardly, and casting an ingot by pouring molten base metal between the base metal faces of the parts which have been placed in an ingot mold. Fig. 3 is a view 40 similar to Fig. 2 indicating that the parts set in the ingot mold have been rolled down be-

fore the base metal is cast therebetween, and Fig. 4 is a cross-sectional view of a rolled bar of base metal faced with stable surface alloy.

In the embodiment illustrated thin sections 10, 10 of easy welding base metal, such as mild steel or iron, are placed back to back in an ingot mold 12 and stable surface alloy material 14 cast about them. The thin sections 10, 10 become highly heated in the casting operation and are firmly and permanently welded to the stable surface alloy material. The base metal sections 10, 10 should be thin enough to take sufficient heat from the molten stable surface material cast thereagainst to overcome the non-welding tendency between such respective materials, and produce the desired good and complete weld therebetween, and should not be so extremely thin as to be melted down by heat so applied. For example, with an ingot mold about 8" x 16" a pair of base metal sections each about 1/4" thick give good results. The inner or meeting surfaces of the base metal sections may advantageously be provided with a surface layer or coating of material adapted to prevent their welding or sticking together, as, for example, by being sooted in a flame of pitch or the like prior to being put in the ingot mold. The other surfaces thereof should preferably be pickled or otherwise cleaned to promote weld formation.

The resulting ingot is cut or broken apart along the line 16 and the resulting ingot parts 18, 18 placed with their base metal faces 101, 101 facing toward one another and additional base metal 20 cast between them, as in an ingot mold 22 (see Fig. 2) or the ingot parts 18, 18 may be subjected to mechanical work as by rolling and the additional base metal 20a cast between the resulting worked down parts 18a, 18a and in contact with the base metal faces 102, 102 thereof (see Fig. 3).

The metal in face parts 101, 102, and the like—preferably identical composition—cast metal 20, 20a become firmly welded together.

in casting even though the complete ingot inserts 18, 18a are of substantial thickness, it being unnecessary to have the ingot inserts of specially thin section for welding the like materials in casting. The rolling down to produce the relatively thin laminated sections 18a while not altogether necessary to produce a weld of the base metals, is of advantage in reduction of cost to produce rolled products having a thin surface layer of stable surface steel.

When ingots so produced are rolled down, bars or other products are obtained as indicated in Fig. 4 having a face or faces of stable surface alloy 14b, 14b and a backing or interior of base metal 20b, which portion 20b, although made up of a plurality of original parts is substantially homogeneous and is closely and firmly welded to the face parts 20 14b of stable surface alloy.

Products so made, in addition to having the surface characteristics of the stable surface alloy used have, of course, the strength and other qualities of the backing material, 25 which preferably constitutes the major part of the product.

I claim:

1. The herein-described process which consists in taking a base metal backing section 30 of reduced thickness compared to the thickness of the backing required for the final product, and having a relatively low heat absorbing capacity, casting a stable surface alloy material in molten condition against one 35 surface of the base metal section in a quantity so that the heat available after absorption of a part thereof is sufficient to weld the two unlike materials together without unduly melting the thin section, and then casting 40 base metal in a molten condition against the opposite surface of the base metal section to weld the same together.

2. The herein-described process which consists in taking a backing section of base metal 45 of reduced thickness compared to the thickness of the backing required in the final product, casting a mass of a stable surface alloy material in molten condition against one surface of the base metal section in a quantity to 50 provide a mass of large heating capacity compared to the heat absorbing capacity of the base metal section so that upon contact of the unlike material sufficient heat is available to weld the two unlike materials together, 55 and then casting base metal in molten condition against the opposite surface of the base metal section to weld the two like materials together, and produce an ingot having a back- 60 ing of base metal of substantial thickness and a face layer of stable surface alloy.

3. The herein-described process which consists in applying a stable surface alloy in a molten condition to one face of the backing section of a base metal of reduced thickness 65 compared to the thickness of the backing re-

quired in the final product and having a relative low heat absorbing capacity compared to the heating capacity of the stable surface alloy so that upon contact of the unlike materials sufficient heat is available after absorption of a part thereof to weld the unlike materials together, and then applying a base metal in a molten condition to the opposite face of said base metal section to weld the like materials together, and increase the thickness 75 of the base metal backing relative to the thickness of the facing of stable surface alloy.

4. The herein-described process which consists in taking a thin section of ferrous base metal and applying to one face thereof a relatively thicker mass of a stable surface iron alloy in a molten condition so that upon contact of the molten mass with the relatively cooler section sufficient heat is available after absorption of a part thereof to cause the two 80 unlike materials to be welded together, and after the composite material so produced has been cooled, applying a like ferrous base metal in a molten condition to the opposite face of said thin section to weld the two latter together and produce a substantially 85 homogeneous backing of ferrous base metal of a thickness greater than that of the layer of stable surface iron alloy welded thereto.

5. The herein-described process which consists in casting stable surface alloy material in molten condition against core forming sections of base metal of reduced thickness compared to the thickness of the core required in the final product, the thickness of the stable 95 surface alloy material and the thicknesses of the sections being proportioned to provide a portion having a large heating capacity and a portion having a relatively small heat absorbing capacity so that upon contact of the unlike materials sufficient heat is available after absorption of part thereof to cause the two unlike materials to be welded together 100 without completely melting the base metal sections, arranging the bi-metallic members 105 so produced with the base metal surfaces thereof facing one another and spaced apart, and casting base metal in molten condition therebetween to weld the molten base metal to the base metal surfaces and increase the thickness of the base metal core relative to the face layers of stable surface alloy material 115 welded thereto.

6. The herein-described process which consists in taking core sections of mild ferrous material of reduced thickness compared to the thickness of the core of the final product and placing the same back to back, casting a mass of a stable surface iron alloy in a molten condition about said sections in a quantity to 120 provide a mass of large heating capacity compared to the heat absorbing capacity of the relatively cool sections so that upon contact of the unlike materials heat is available after absorption of a part thereof to weld the un- 125 130

like materials together, separating bi-metallic parts of the resulting product and arranging the same with the faces of mild ferrous material facing one another and spaced 5 apart, and casting mild ferrous material in molten condition therebetween to weld the like materials together, and produce an ingot having a relatively thick intermediate portion of substantially homogeneous mild ferrous material and face layers of stable surface iron alloy.

In testimony whereof, I have signed my name hereto.

PERCY A. E. ARMSTRONG.

15

20

25

30

35

40

45

50

55

60